

[54] **LOW-WEAR GREASE FOR JOURNAL BEARINGS**

[75] Inventor: **Ruel M. Donaho, Jr.**, Houston, Tex.

[73] Assignee: **Hughes Tool Company**, Houston, Tex.

[22] Filed: **Dec. 4, 1974**

[21] Appl. No.: **529,302**

**Related U.S. Application Data**

[63] Continuation of Ser. No. 292,021, Sept. 25, 1972, abandoned.

[52] **U.S. Cl.**..... **252/18; 252/25**

[51] **Int. Cl.<sup>2</sup>** **C10M 3/18; C10M 5/14; C10M 7/20; C10M 7/24**

[58] **Field of Search**..... **252/18, 25**

[56] **References Cited**

**UNITED STATES PATENTS**

|           |         |                     |        |
|-----------|---------|---------------------|--------|
| 3,194,760 | 7/1965  | Davis .....         | 252/18 |
| 3,223,626 | 12/1965 | Murphy et al. ....  | 252/25 |
| 3,396,108 | 8/1968  | Caruso.....         | 252/18 |
| 3,472,770 | 10/1969 | Preston et al. .... | 252/18 |

*Primary Examiner*—Delbert E. Gantz

*Assistant Examiner*—I. Vaughn

*Attorney, Agent, or Firm*—Robert A. Felsman

[57] **ABSTRACT**

A low-wear grease for journal bearings characterized by a high temperature, multi-purpose heavy duty hydrocarbonaceous lubricant that is thickened by calcium acetate complex to form a lubricating grease having an ASTM worked penetration no less than 265; and molybdenum disulfide and a selected class of metallic oxide in effective and synergistic amounts. Surprisingly, better lubrication is provided when the molybdenum disulfide particles are non-uniform in size so they have a range of sizes, including some fine and some relatively coarse but are small enough to pass 100 percent through a 100 mesh screen, and 85 percent through a 325 mesh screen. The metallic oxide is either antimony trioxide or a mixture of substantially equal parts of antimony trioxide, zinc oxide, lead oxide, nickel oxide, tungsten trioxide, vanadium pentoxide and copper oxide. The particles of the metallic oxide are small enough to pass 90 percent through a 325 mesh screen. All particles are uniformly dispersed in the thickened, heavy duty lubricating grease.

11 Claims, No Drawings

## LOW-WEAR GREASE FOR JOURNAL BEARINGS

This is a continuation, of application Ser. No. 292,021, filed Sept. 25, 1972 and now abandoned.

## BACKGROUND OF THE INVENTION

## 1. Field of the Invention

This invention relates to new grease compositions; and, more particularly, to improved, low-wear grease for heavy duty, high temperature applications, such as for journal bearings on bits drilling into hot subterranean formations.

## 2. Description of the Prior Art

Complex-thickened greases are well known in the art. For example, an excellent discussion is contained in the ENCYCLOPEDIA OF CHEMICAL TECHNOLOGY, KIRK-Othmer, Second Edition, A. Standen, Editor, Interscience Publishers, John Wiley & Sons, Inc., New York, N.Y., 1967, pages 582-587. Also, it is known to employ certain complexes; such as, the calcium-acetate-containing complexes and the lithium-hydroxy-stearate-containing complexes; to provide high temperature stability and maintain lubrication properties at the high temperatures to which the 15 greases may be subjected.

Lubricating a drill bit drilling in hot (frequently above 300°F) subterranean formations is one of the most severe and demanding set of conditions ever posed for a lubricant. The drilling takes place in an abrasive atmosphere of drilling mud and rock particles thousands of feet from the engineer or supervisor, who does not have benefit of oil pressure gauges or temperature sensors at the surfaces to be lubricated. The lubricant should have properties that enable flow through 20 passageways to the surfaces to be lubricated and that prevent solid lubricant particles from settling out.

The best available lubricants heretofore have not satisfactorily minimized wear under the heavy load conditions encountered by earth boring drill bits having friction bearings.

The prior art shows solid extreme pressure (EP) additives have been employed to attempt to enhance the lubrication properties of oils and greases. For example, molybdenum disulfide has been used in a wide 45 variety of lubricants, as noted in U.S. Pat. Nos. 3,062,741, 3,170,878, 3,281,355 and 3,384,582. The prior art has taught, however, that the molybdenum disulfide should comprise fine particles having an average diameter less than 10 microns and some prefer less than 2 microns.

Also, it is known to include metallic oxides like zinc oxide in other lubrication oils. Moreover, U.S. Pat. No. 2,736,700 describes the use of molybdenum disulfide and a metallic oxide, such as fumed lead oxide and zinc oxide in a ratio of 2 parts molybdenum disulfide to 1 part metallic oxide, in a paint-on composition, or bonded lubricant, containing a lacquer drying agent. The bonded lubricant is described for drawing tough metals, such as uranium, thorium, zinc and titanium. Such bonded lubricants are inadequate and could not be employed in the low-wear, heavily loaded applications for which this invention was engineered.

Insofar as I am aware, the prior art has not provided a heavy duty lubricant employing a hydrocarbonaceous grease that is calcium acetate complex thickened for temperature stability and that has the superior lubricating properties of this invention; particularly, that could

be employed in the application of lubricating journal bearings in bits drilling in an abrasive atmosphere thousands of feet from the engineer or supervisor; or under conditions that are similarly severe and demanding of 5 the grease.

## SUMMARY OF THE INVENTION

Accordingly, it is a primary object of this invention to provide a grease that is temperature stable and that can 10 be employed under severe and demanding conditions; such as, for lubricating journal bearings of bits penetrating subterranean formations; by providing a degree of protection not heretofore available at the extreme pressure, high temperature atmosphere conditions to 15 which the lubricant will be subjected.

It is a particular object of this invention to provide a grease that has physical properties, such as a worked penetration, sufficient to flow to the surfaces to be lubricated; and not flow out of the bit but to provide 20 lubrication and protection greater than available heretofore at temperatures in excess of 300°F.

These and other objects will become apparent from the following descriptive matter.

In accordance with this invention, the superior grease 25 consists essentially of a substantially uniform dispersion including:

a. a multi-purpose heavy duty hydrocarbonaceous lubricant thickened by a calcium acetate complex to form a heavy duty lubricating grease that is stable at 30 high temperatures and that has an American Society for Testing Materials (ASTM) worked penetration no less than 265; and effective and synergistic amounts of the solid additives of:

35 b. molybdenum disulfide ( $MoS_2$ ) powder; and c. metallic oxide powder; the metallic oxide being selected from the group consisting of antimony trioxide ( $Sb_2O_3$ ); and a mixture of substantially equal parts of antimony trioxide, zinc oxide ( $ZnO$ ), lead oxide ( $PbO$ ), nickel oxide ( $Ni_2O_3$ ), tungsten trioxide ( $WO_3$ ), vanadium pentoxide ( $V_2O_5$ ) and copper oxide ( $CuO/Cu_2O$ ).

The effective and synergistic amounts of the powdered solid additives in the lubricating grease preferably includes at least 7 percent by weight of molybdenum disulfide and at least 5 percent by weight of the metallic oxide when employed in a downhole bit. The percent by weight is based on the final weight of grease. The powder is also preferably made up of a range of non-uniform particle sizes, as delineated hereinafter.

50 A particularly preferred grease consists essentially of the lubricating grease containing 11-20 percent by weight of the molybdenum disulfide and 5-20 percent by weight of the metallic oxide. Other non-detrimental additives, such as graphite, may be employed if desired.

## 55 DESCRIPTION OF PREFERRED EMBODIMENT(S)

The grease of this invention, with its superior lubrication properties, is prepared by dispersing uniformly in a conventional high temperature, calcium acetate complex thickened lubricating grease, the desired effective and synergistic amounts of molybdenum disulfide and the metallic oxide chosen. The molybdenum disulfide and the metallic oxide additives can be incorporated into the grease at almost any stage in the manufacture 60 of the final product, dependent upon the convenience with respect to the particular grease plant. For example, they can be incorporated when the thickener is added; or, ordinarily, they can be incorporated at some

stage in the handling of the semi-finished product. The important feature is that sufficient mixing should be employed; as by working, homogenizing, or otherwise; to secure a complete, uniform, and thorough dispersion of the particles of the molybdenum disulfide and the metallic oxide throughout the grease.

Considering the constituents of the grease, the "lubricating grease", as used herein, denotes a high temperature, multi-purpose heavy duty hydrocarbonaceous lubricant that has been thickened by a calcium acetate complex. The lubricating grease has an ASTM D-217 test, in depth of penetration in tenths of a millimeter in five seconds at 77°F, no less than 265. The lubricating grease has a National Lubricating Grease Institute (NLGI) classification of less than class 3 to effect the requisite flow through passageways to reach and lubricate the surfaces of interfacing elements, such as bearings. Thus, the lubricating grease falls in the NLGI class 00, class 0, class 1, or class 2. The methods of dispersion and the NLGI table of classification, including physical properties for the classes, is included in the above-referenced ENCYCLOPEDIA OF CHEMICAL TECHNOLOGY; for example, the NLGI classification table is included at page 586. Accordingly, this voluminous material need not be duplicated herein. The greases employ a calcium complex type of thickener that contains calcium acetate as a primary ingredient. A suitable lubricating grease is the Amdex No. 0 EP or the No. 1 EP, available from American Oil Company. The satisfactory Amdex greases have the specifications set forth in Table I.

Table I

| Property                            | Amdex Grease<br>No. 0 EP | Amdex Grease<br>No. 1 EP |
|-------------------------------------|--------------------------|--------------------------|
| Worked Penetration, 60 strokes      | 369                      | 325                      |
| Worked Penetration, 100,000 strokes | 382                      | 343                      |
| Viscosity of Oil at 100°F, SUS      | 900                      | 900                      |
| Viscosity index of oil              | 90                       | 90                       |
| Timken EP, lbs. pass                | 55                       | 55                       |
| Dropping point, °F                  | 500+                     | 500+                     |
| Bearing rust protection test        | No. 1                    | No. 1                    |
| Bomb oxidation, psi* drop/100 hrs.  | 3                        | 3                        |
| Copper corrosion                    | Pass                     | Pass                     |
| Roll stability, 20 hrs., % change   | +2.6                     | +5.1                     |
| Oil separation, 24 hrs. at 210°F %  | 2.9                      | 2.0                      |

\*psi — pounds per square inch

lbs. — pounds

hrs. — hours

SUS — Saybolt universal seconds

% — percent

Other calcium-acetate-complex thickened greases; such as those described in U.S. Pat. No. 2,999,065 and U.S. Pat. No. 2,999,066 should be satisfactory, although they have not been tested. In any event, the lubricating grease should have lubricating properties, before addition of the solid additives, sufficient to provide a Shell 4-ball EP scar diameter of 1.3 millimeters (mm) maximum after five minutes (min.) at 900 revolutions per minute (rpm) under 200 kilogram (kg).

The particulate molybdenum disulfide, as indicated hereinbefore, is small enough to pass 100 percent through a 100 mesh per inch screen, and 85 percent through a 325 mesh screen such that it may be easily substantially uniformly dispersed throughout the lubricating grease. The percents are by weight. I have found, surprisingly, that molybdenum disulfide having a complete range of particle sizes, some fine and some coarse, affords better extreme pressure lubrication properties than classified, relatively uniform sizes of

less than 10 microns, or even less than 2 microns, as taught by the prior art. A satisfactory commercial grade of molybdenum disulfide is Esco, available from Dow Corning as No. 3490 molybdenum disulfide that is not size-segregated and has the desired range of particle sizes. The Esco molybdenum disulfide meets the foregoing criteria and has about 2-4 percent retained on a 200 mesh screen.

The particulate metallic oxide is small enough to pass 100 percent through a 100 mesh screen and 90 percent through a 325 mesh screen such that the metallic oxide may be readily substantially uniformly dispersed in the lubricating grease. A satisfactory metallic oxide comprises a mixture of substantially equal parts of antimony trioxide, zinc oxide, lead oxide, nickel oxide, tungsten trioxide, vanadium pentoxide and copper oxide. I have found it preferable, however, to employ the single oxide of antimony trioxide to obtain superior results without the bother of having to blend the mixture of oxides. A satisfactory commercial grade of antimony oxide is White Star M, available from Harshaw Chemical Company as a fine powder. The satisfactory antimony trioxide has the properties set forth in Table II.

Table II

| Chemical or Element              | Specifications  |      |
|----------------------------------|-----------------|------|
| Sb <sub>2</sub> O <sub>3</sub> * | 99.00%          | min. |
| Pb*                              | 0.05%           | max. |
| Cu*                              | 0.004%          | max. |
| Ni*                              | 0.004%          | max. |
| As*                              | 0.05%           | max. |
| Fe*                              | 0.007%          | max. |
| SO <sub>4</sub> *                | 0.01%           | max. |
| Physical properties (typical)    |                 |      |
| Specific gravity                 | 5.72            |      |
| Oil absorption                   | 10.0            |      |
| Reflectance in Oil               | 92%             |      |
| Color (mass tone)                | Excellent white |      |
| Tint Strength                    | Pigment quality |      |
| Residue on 325 mesh              | 0.022%          |      |

\*Symbols used in accordance with the Periodic Table

A grease that is minimally satisfactory for a drill bit is provided by the inclusion of as little as 7 percent molybdenum disulfide and 5 percent metallic oxide into the lubricating grease. It is preferred, however, that an amount within the range illustrated in Table III be employed. The amounts in Table III are percent by weight based on a uniform dispersion in the final grease composition and are incorporated into the lubricating grease described hereinbefore.

TABLE III

|              | MoS <sub>2</sub> | Metallic Oxides | Graphite | Total |
|--------------|------------------|-----------------|----------|-------|
| Lower limits | 11%              | 5%              | 0%       | 16%   |
| Optimum      | 13               | 7               | 0        | 20    |
| Upper limits | 20               | 20              | 5        | 36    |

As noted from the total percentage in Table III, the maximum amount of molybdenum disulfide would not be employed with the maximum amount of the metallic oxides, since no more than 36 percent of solid EP additives is employed, preferably.

The following examples illustrate satisfactory greases prepared in accordance with this invention. Different size batches were prepared and tested on the Shell 4-ball EP tester. The Shell 4-ball EP tester has been demonstrated to give excellent results in testing a lubricant for extremely severe and demanding steel-sliding-on-steel applications. The Shell 4-ball EP tester has been described in the literature and is well known so it need not be described herein. Basically, a lubricant is tested in contact with four balls, the top ball being rotated while loaded. After a predetermined length of time the diameter of the wear scar is measured. The smaller the scar dimension is, the better the lubricant is. Finally, a table, Table IV, summarizes several of the many compositions, including tests on compositions similar to those delineated in the Examples, tried in arriving at the grease of this invention.

#### EXAMPLE I

This example illustrates the best grease yet prepared.

Respective amounts of molybdenum disulfide and antimony trioxide were added to the Amdex 0 EP lubricating grease to form a grease that had 14 percent molybdenum disulfide by weight and 7 percent antimony trioxide by weight with 79 percent Amdex 0 EP.

A similar grease was formed by adding 13 percent molybdenum disulfide and 7 percent antimony trioxide

to 80 percent of Amdex 0 EP lubricating grease effected a final product that was almost equally as satisfactory.

#### EXAMPLE II

Another grease that performed satisfactorily was made by adding respective amounts of molybdenum disulfide and a mixture of substantially equal parts of metallic oxides to the Amdex 0 EP lubricating grease to form a uniform admixture containing 14 percent molybdenum disulfide and 7 percent metallic oxides. The metallic oxides had substantially equal parts of antimony trioxide, zinc oxide, lead oxide, nickel oxide, tungsten trioxide, vanadium pentoxide and the copper oxides. The copper oxides comprised both cuprous and cupric oxide in about equal portions, although they combined to form an amount equal to that of the respective other oxides employed. This grease was almost as good as those of Example 1, as shown in Table IV.

#### EXAMPLE III

In this example, graphite in the same range of particle sizes as described with respect to molybdenum disulfide and the antimony trioxide were added to a variety of grease formulations. In general, the substitution of the graphite for either the molybdenum disulfide or the antimony trioxide resulted in an inferior grease. The graphite could be included, however, in addition to the satisfactory effective and synergistic amounts of the molybdenum disulfide and the metallic oxide, such as antimony trioxide, without adversely affecting the properties of the grease. The data are summarized in Table IV hereinafter.

Table IV summarizes a variety of compositions that were tried and illustrates some satisfactory and unsatisfactory compositions that were surprising. Table IV summarizes the results in terms of the scar diameters obtained in the Shell 4-ball EP tests on different greases, and inspection of worn journal bearings after a simulated run, referred to as "Journal Bearing Test" in Table IV.

Table IV

| Formulation and Remarks                                                                                                                                | Weight % Solid EP Additives |                                |            |          | Avg. EP Scar Diameter (mm) |                   |                    | Journal Bearing Test |
|--------------------------------------------------------------------------------------------------------------------------------------------------------|-----------------------------|--------------------------------|------------|----------|----------------------------|-------------------|--------------------|----------------------|
|                                                                                                                                                        | MoS <sub>2</sub>            | Sb <sub>2</sub> O <sub>3</sub> | Oxide Mix* | Graphite | 900 rpm<br>500 KG          | 900 rpm<br>550 KG | 1800 rpm<br>300 KG |                      |
| 1. grease employing lithium hydroxy stearate thickener; large scar diameter                                                                            | 14                          | 7                              |            |          | 1.97**                     |                   |                    | W                    |
| 2. same grease, additional additives, no improvement                                                                                                   | 15                          | 15                             |            |          | 1.96**                     |                   |                    | W                    |
| 3. Amdex 0 EP + MoS <sub>2</sub>                                                                                                                       | 7                           |                                |            |          | 1.49                       | 1.62              |                    | W, 1.43              |
| 4. Amdex 0 EP + additional MoS <sub>2</sub> ; no improvement                                                                                           | 19 to 24                    |                                |            |          | 1.56                       | 1.55              | 1.44               |                      |
| 5. Amdex 0 EP + MoS <sub>2</sub> + small amount Sb <sub>2</sub> O <sub>3</sub> , 3% Sb <sub>2</sub> O <sub>3</sub> is better than 15% MoS <sub>2</sub> | 7                           | 3                              |            |          | 1.51                       | 1.57              |                    |                      |
| 6. Amdex 0 EP + MoS <sub>2</sub> + more Sb <sub>2</sub> O <sub>3</sub> ; appreciable improvement                                                       | 7                           | 5 to 10                        |            |          | 1.43                       | 1.56              | 1.39               |                      |
| 7. 6 + graphite; graphite apparently not detrimental                                                                                                   | 7                           | 7                              |            | 7        | 1.44                       | 1.55              |                    |                      |
| 8. Amdex 0 EP, preferred composition, appreciable improvement over other compositions tested                                                           | 11 to 16                    | 5 to 20                        |            |          | 1.35                       | 1.49              | 1.25               | Very good            |
| 9. 8 + graphite; graphite apparently not detrimental                                                                                                   | 13                          | 7.5                            |            | 5        | 1.34**                     |                   | 1.25               |                      |
| 10. mixed oxides* in lieu of Sb <sub>2</sub> O <sub>3</sub> ; almost as good as Sb <sub>2</sub> O <sub>3</sub>                                         | 13                          | 7                              |            |          | 1.38                       | 1.47              |                    | Good                 |
| 11. graphite in lieu of MoS <sub>2</sub> ; bearing galled                                                                                              | 6                           |                                |            | 5        | 9.5                        | 1.35              | 1.49               | Galled               |
| 12. less oxides than 11; bearing galled                                                                                                                | 10                          |                                |            | 3.5      | 5                          | 1.38              | 1.49               | Galled               |

\*Equal parts (by weight): Sb<sub>2</sub>O<sub>3</sub> + ZnO + PbO + Ni<sub>2</sub>O<sub>3</sub> + WO<sub>3</sub> + V<sub>2</sub>O<sub>5</sub> + (CuO + Cu<sub>2</sub>O)

\*\*400 KG load instead of 500 KG W = Welded during 4-ball EP test

As can be seen from Table IV, there are effective and synergistic amounts of the solid additives. For example, run 5 indicates that 3% of the metallic oxide added to at least 7% of  $\text{MoS}_2$  is better than 15% of additional  $\text{MoS}_2$ . Adding a little more metallic oxide up to 5% effected significant improvement. Attempts to substitute graphite for one or more of the ingredients did not produce a satisfactory grease. The addition of the  $\text{MoS}_2$  and  $\text{Sb}_2\text{O}_3$  did not sufficiently improve the performance of the grease that had been thickened with lithium hydroxy stearate (see runs 1. and 2.), as they did for the calcium-acetate-complex-thickened grease. This invention takes advantage of the surprisingly low wear obtained using the combination calcium-acetate-complex-thickened grease and the minimum concentration of the  $\text{MoS}_2$  and the metallic oxides uniformly dispersed therein. In fact, by using the delineated effective and synergistic amounts of the solid additives, the final grease will lubricate sufficiently to effect a Shell 4-ball EP scar diameter of about 1.4 millimeters maximum after five minutes at 900 revolutions per minute under 500 kilograms load. This represents outstanding performance.

Having thus described the invention, it will be understood that such description has been given by way of illustration and example and not by way of limitation, reference for the latter purpose being had to the appended claims.

What is claimed is:

1. A heavy duty lubricating grease consisting essentially of a substantially uniform dispersion including:  
 a. a multi-purpose heavy duty hydrocarbonaceous lubricant thickened by a calcium acetate complex to form a lubricating grease that is stable at high temperature and that has an ASTM worked penetration of no less than 265; and effective and synergistic amounts of:  
 b. powdered molybdenum disulfide; and  
 c. powdered metallic oxide; said metallic oxide being selected from the group consisting of antimony trioxide; and a mixture of substantially equal parts of antimony trioxide, zinc oxide, lead oxide, nickel oxide, tungsten trioxide, vanadium pentoxide and copper oxide;

such that said heavy duty lubricating grease can be prepared to have a Shell 4-ball EP scar diameter of about 1.4 millimeters maximum after 5 minutes at 900 revolutions per minute at 500 kilograms load.

2. A heavy duty lubricating grease consisting essentially of a substantially uniform dispersion including:

a. a multi-purpose heavy duty hydrocarbonaceous lubricant thickened by a calcium acetate complex to form a lubricating grease that is stable at high temperatures and has an ASTM worked penetration of no less than 265; and effective and synergistic amounts of:  
 b. particles of molybdenum disulfide that are small enough to pass 100 percent through a 100 mesh screen and 85 percent through a 325 mesh screen,  
 c. particles of antimony trioxide that are small enough to pass 100 percent through a 100 mesh screen and 90 percent through a 325 mesh screen,  
 such that said heavy duty lubricating grease can be prepared to have a Shell 4-ball EP scar diameter of about 1.4 millimeters maximum after 5 minutes at 900 revolutions per minute under 500 kilograms load.

3. A heavy duty lubricating grease consisting essentially of a substantially uniform dispersion including:

5 a. a multi-purpose heavy duty hydrocarbonaceous lubricant thickened by a calcium acetate complex to form a lubricating grease that is stable at high temperatures and has an ASTM worked penetration of no less than 265; and effective and synergistic amounts of:

b. particles of molybdenum disulfide that are small enough to pass 100 percent through a 100 mesh screen and 85 percent through a 325 mesh screen;  
 c. particles of metallic oxide consisting of a mixture of substantially equal parts of antimony trioxide, zinc oxide, lead oxide, nickel oxide, tungsten trioxide, vanadium pentoxide and copper oxide; said metallic oxide particles being small enough to pass 100 percent through a 100 mesh screen and 90 percent through a 325 mesh screen;

10 such that said heavy duty lubricating grease can be prepared to have a Shell 4-ball EP scar diameter of about 1.4 millimeters maximum after 5 minutes at 900 revolutions per minute under 500 kilograms load.

15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980 9985 9990 9995 10000 10005 10010 10015 10020 10025 10030 10035 10040 10045 10050 10055 10060 10065 10070 10075 10080 10085 10090 10095 10100 10105 10110 10115 10120 10125 10130 10135 10140 101

disulfide is present in an amount of about 13 percent by weight.

9. The grease of claim 4 wherein said metallic oxide is present in an amount within the range of 5-20 percent by weight.

10. The grease of claim 9 wherein said metallic oxide is present in an amount of about 7 percent by weight.

11. The grease of claim 4 wherein said molybdenum disulfide is present as a solid EP additive in an amount

10  
within the range of 11-20 percent by weight; said metallic oxide is present as a solid EP additive in an amount within the range of 5-20 percent by weight; and wherein graphite, as another solid EP additive, is present in an amount of no more than 5 percent by weight; and the total amount of EP solid additives is no more than 36 percent by weight.

\* \* \* \* \*